

[54] PROCEDURE FOR MANUFACTURING HIGH QUALITY ZINC POWDER

[76] Inventor: Tomas Perez Calleja, S. Gervasio s/n (Vellaverde bajo), Madrid, Spain

[22] Filed: May 10, 1971

[21] Appl. No.: 141,770

[30] Foreign Application Priority Data

May 18, 1970 Spain ..... 379,780

[52] U.S. Cl. ..... 75/0.5 B, 75/88

[51] Int. Cl. ..... B22f 9/00

[58] Field of Search ..... 75/88, .5 B

[56] References Cited

UNITED STATES PATENTS

|           |         |               |         |
|-----------|---------|---------------|---------|
| 1,287,949 | 12/1918 | Fricker       | 75/88   |
| 905,753   | 12/1908 | Shortman      | 75/88   |
| 1,233,652 | 7/1917  | DeBavay       | 75/88   |
| 1,495,961 | 5/1924  | Newell et al. | 75/88   |
| 2,007,027 | 7/1935  | Schulze       | 75/88   |
| 500,436   | 6/1893  | Smith         | 75/88 X |
| 1,980,480 | 11/1934 | Ginder et al. | 75/88   |
| 2,823,111 | 2/1958  | Davey et al.  | 75/88   |

3,563,727 2/1971 Webb ..... 75/88 UX  
1,994,345 3/1935 Holstein et al. ..... 75/88

Primary Examiner—L. Dewayne Rutledge

Assistant Examiner—M. J. Andrews

Attorney—Wenderoth, Lind & Ponack

[57] ABSTRACT

A method of manufacturing high quality zinc powder in an independent grouping of small modular components, each having a combination oven and condensation chamber. There is a melting crucible and a retort or zinc vaporizing crucible inside the oven and the condensation chamber has several independent deposits in the lower area where condensed zinc particles settle and are later collected. A device in the condensation chamber acts as a safety valve which eliminates the risk of explosion when an abnormal reaction occurs inside the chamber. A device in the condensation chamber functions as a cleanser for zinc oxide to control not very violent abnormal reactions. A filtering device can be installed between the steaming retort or crucible and the condensation chamber which eliminates impurities in the zinc utilized.

1 Claim, 7 Drawing Figures



PATENTED OCT 30 1973

3,768,995

SHEET 1 OF 5



FIG - 1



FIG - 2



FIG - 3

Tomas PEREZ CALLEJA, Inventor

By, *Wendell W. Lind & Preach*

Attorneys

PATENTED OCT 30 1973

3,768,995

SHEET 2 OF 5



FIG-4

Tomas PEREZ CALLEJA, Inventor

By, *Wendt, Lind & Ponack*  
Attorneys

PATENTED OCT 30 1973

3,768,995

SHEET 3 OF 5



FIG - 5

Tomas PEREZ CALLEJA, Inventor

By, *Wendell Lind Ponack*

Attorneys

PATENTED OCT 30 1973

3,768,995

SHEET 4 OF 5



FIG-6

Tomas PEREZ CALLEJA, Inventor

BY *Wendworth, Lind & Roach*  
Attorneys

PATENTED OCT 30 1973

3,768,995

SHEET 5 OF 5



FIG-7

Tomas PEREZ CALLEJA, Inventor

By *Wendell Lind Ponack*  
Attorneys

## PROCEDURE FOR MANUFACTURING HIGH QUALITY ZINC POWDER

### BACKGROUND OF THE INVENTION

This invention relates to a procedure for manufacturing high quality zinc powder.

Production of high quality zinc powder is currently carried out by procedures requiring installations of certain dimensional characteristics, generally quite large and costly, so that when production of zinc powder is required to exceed that which has been preestablished, another plant of equal characteristics is necessary. The cost of such manufacture increases substantially since the new plant is as costly as the first one.

### OBJECTS AND BRIEF DESCRIPTION OF THE INVENTION

This difficulty is satisfactorily resolved by means of this invention which consists fundamentally in grouping various small independent and inexpensive modular components which, assembled in a battery, may easily be shut down or placed in operation and therefore, production of zinc powder can be reduced or increased without resulting in a substantially higher cost of the product obtained.

A primary object of the present invention is the provision of an installation for manufacturing high quality zinc powder at a very low cost.

A further object of the present invention is the provision of a process for eliminating impurities if zinc containing the same is utilized.

A further object of the present invention is the provision of a process employing a safety device to prevent explosions which would destroy the installation.

A still further object is the provision of a process which allows for eliminating a very high percentage of zinc oxide (ZnO) in the zinc powder produced, whereby it is possible to compete advantageously with any installation. This process prevents the operation of the safety device when an abnormal, not very violent reaction, occurs in the condensation chamber.

The advantages and results obtained by employing the present invention are as follows:

A. Very low cost of installation, and with regard to the quality and quantity of zinc powder produced, there is an important difference in price between product produced by the present invention and prior processes.

B. It is possible to expand the installation indefinitely without affecting other assembled modular components, due to their total independence, thereby resulting in a very low additional cost.

C. It is possible to produce a quality of zinc powder with a minimum of 95% metal zinc.

D. The elimination of explosion risks is possible.

E. The practical elimination of zinc oxide (ZnO) content in the finished product is made possible.

F. Absolute simplicity in assembly, operation and maintenance of the system are made possible.

G. Operating and maintenance expenses are very low.

H. According to this invention, production of zinc powder and never totally stop for technical reasons, because the installation consists of an assembly of modular components totally independent of each other. Each of the components need not be inoperative in excess of eight days, a more than sufficient time for re-

placement of worn parts and, consequently, production is not interrupted for long periods as is the case with other installations. According to the invention, with constant production, the maximum inconvenience which might occur is that it might become necessary to stop certain of the modular components and momentarily reduce production.

I. Continuity of the system due to its heat loads is made possible.

J. Minimum production of each modular component is in excess of 1,000 kilos daily.

The procedure observed for production of high quality zinc powder on the basis of zinc according to this invention is as follows:

15 The zinc is melted and subsequently loaded into a retort or crucible, the zinc then being vaporized in the retort or crucible proper. This vapor passes through a device for eliminating impurities and then to a condensation chamber. Vapor in this chamber is deposited as zinc powder in receptacles. These receptacles are removed as they are filled, and replaced by empty receptacles. Later the zinc powder obtained is put through a sieve. When the zinc in the retort or crucible is almost consumed, the process is initiated again without interrupting its continuity.

### BRIEF DESCRIPTION OF THE DRAWINGS

With a view to graphically clarifying the idea described, reference will be made to the following detailed description as well as the accompanying drawings wherein:

FIG. 1 is a perspective view of a crucible for melting the zinc.

FIG. 2 is a perspective view of a retort or crucible in which zinc is vaporized.

FIG. 3 is a perspective view of a chamber for eliminating impurities from the zinc.

FIG. 4 is a perspective view of a chamber where zinc is condensed and of the deposits where the product is collected.

FIG. 5 is a partially sectioned schematic view of one of the modular components of the installation.

FIG. 6 is a schematic view of the same component from another point located 90° in relation to the above.

FIG. 7 is a view similar to that shown in FIG. 6 but in which the modular component has no crucible for melting the zinc.

### DETAILED DESCRIPTION OF THE INVENTION

With reference to the drawings it is observed that a melting crucible 1 for melting the zinc, is situated inside an oven 9 having a chimney 10, but farther from burners (not shown) than a retort or crucible 2, where the zinc is vaporized. The temperature in the vicinity of the retort 2 is in excess of the boiling point of the zinc. 2' is an addition to the retort, and 2'' is a retort cover.

As shown in FIG. 7, the zinc need not be melted in the modular component shown, but may arrive at the retort 2, already melted, in order to continue the process from there.

In the case represented in FIG. 6 as well as that in FIG. 7, the melted zinc is vaporized in retort 2 and thus passes to chamber 3, equipped with an intake conduit fitted to the upper part of 2', and with an outlet fitted to condensation chamber 4. Inside chamber 3 for eliminating impurities from the zinc vapor there is coke, whereby any possible impurities are retained and do

not pass to condensation chamber 4. As shown in FIGS. 3 and 5 the filter inlet is positioned lower than the filter outlet. Thus, any impurities, such as lead, in filter 3 will drop back to retort 2, due to their heavier weight.

When the zinc metal utilized contains few impurities it requires no device such as chamber 3, and in this case the zinc vapor passes directly from the vaporizing retort 2, to condensation chamber 4.

Pure zinc vapor passes to the condensation chamber 4, settles in powdered form in each of the deposits or receptacles 5. These deposits 5 are removed as they are filled, and are replaced by empty receptacles so that periodic collection of zinc powder may continue.

Formation of explosions inside the condensation chamber 4, due to violent reaction between oxygen and zinc is totally controlled by a safety device 6, provided in the upper part of condensation chamber 4. A purging device 7 is fitted in the lower part of the chamber 4 to control and expel the zinc oxide resulting in chamber 4, and when a not very violent abnormal reaction occurs in chamber 4, device 7 controls the reaction and prevents device 6 from operating.

I claim:

1. Process for producing high quality zinc powder comprising:

5

10

15

20

25

30

35

40

45

50

55

60

65

- a. pouring melted zinc into a retort;
- b. heating said retort until said melted zinc boils, thus forming vaporized zinc;
- c. passing said vaporized zinc through a filter such that the filter inlet is located in a plane lower than the filter outlet, thereby causing impurities in said vaporized zinc to be retained in said filter;
- d. passing said vaporized zinc from said filter to a chamber, thus producing expansion of said vaporized zinc, thus initially forming zinc oxide from reaction with oxygen within said chamber;
- e. purging said zinc oxide from said chamber by opening a discharge valve;
- f. closing said discharge valve when all of said zinc oxide is purged from said chamber, and thereafter forming zinc powder from expansion of said vaporized zinc in said chamber;
- g. allowing said zinc powder to constantly drop by gravity into vessels situated below said chamber; and
- h. providing a safety relief plate in the upper part of said chamber to avoid explosions when high pressures may eventually be produced within said chamber.

\* \* \* \* \*

25

30

35

40

45

50

55

60

65